

June 6, 1939.

F. HANSGIRG.

2,160,969

PROCESS OF PRODUCING PURE MAGNESIUM

Original Filed Feb. 3, 1933

3 Sheets-Sheet 1



WITNESSES

O. B. Wallace.

J. B. Flick.

BY

Fritz Hansgirg  
Brown, Critchlow & Flick  
his ATTORNEYS

June 6, 1939.

F. HANSGIRG

2,160,969

PROCESS OF PRODUCING PURE MAGNESIUM

Original Filed Feb. 3, 1933 3 Sheets-Sheet 2

*Fig. 2.*



WITNESSES

*A.B. Wallace.*  
*J.B. Flex.*

INVENTOR.

*Fritz Hansgirg*  
BY *Brown, Critchlow & Flex*  
his ATTORNEYS

June 6, 1939.

F. HANSGIRG

2,160,969

## PROCESS OF PRODUCING PURE MAGNESIUM

Original Filed Feb. 3, 1933

3 Sheets-Sheet 3

Fig. 3.



**WITNESSES**

A. B. Wallace.  
J. B. Thix

INVENTOR.

BY *Fritz Hausinger*  
*Brown, Cuttler & Haas*  
*his ATTORNEYS.*

## UNITED STATES PATENT OFFICE

2,160,969

## PROCESS OF PRODUCING PURE MAGNESIUM

Fritz Hansgirg, Radenthein, Austria, assignor to  
American Magnesium Metals Corporation,  
Pittsburgh, Pa., a corporation of Delaware

Original application February 3, 1933, Serial No.  
655,067. Divided and this application November  
20, 1934, Serial No. 753,890

1 Claim. (Cl. 75—67)

This invention relates to a process of producing substantially pure magnesium.

Like all solid substances having a considerable vapor tension even below their melting point, metallic magnesium displays a tendency to pass directly from the condition of vapor into the solid state, without the occurrence of a liquid phase. It has therefore been repeatedly recommended to purify magnesium by sublimation or to produce it in crystalline form, from magnesium-containing starting materials, a process which, however, is attended *inter alia*, with the drawback, in operating on a technical scale, that it can only be performed in a periodic manner. On the other hand, the distillation of magnesium has hitherto encountered serious difficulties.

One object of the present invention is to separate substantially pure magnesium from non-volatile concomitant substances.

Another object of my invention is to enable magnesium to be distilled so as to condense the distillate as a liquid deposit.

A further object of the invention is to provide a process for the distillation of material containing metallic magnesium which can be carried on continuously.

My process comprises passing crude metallic magnesium, or material high in magnesium, continuously through a heated zone, in order to heat it to a temperature above the melting point, and preferably in the neighborhood of the boiling point of magnesium, the disengaged vapors being carried by an inert or reducing gas, through an interposed filter, into the condensing zone, the vapors being prevented from cooling below the solidification point of the magnesium, by being heated on their way to the condensing zone, and being thereafter suddenly cooled to the condensation point. The filtration serves to remove contaminating particles of dust from the metallic vapors. This process is performed at reduced pressures.

While various types of apparatus might be employed for carrying out this process, a typical apparatus according to the present invention consists substantially of an externally heated distillation chamber which is provided with a conveyor and connected, at each end, with lock chambers, through a stock vessel or collector, and also with a condenser from which the molten magnesium runs off into a collector, for example, through a barometric outlet, a filter being interposed between the said distillation chamber and the said condenser. The still, filter, condenser, outlet and receiver are preferably housed in a

common heating chamber, such as an electric radiation furnace.

In order to render the filtration process continuous, it is advisable to employ a filter of loose, granular material, piled up loosely between an intake and closable outlet, in the passage connecting the still chamber with the condenser.

In a preferred embodiment of apparatus for carrying out the invention, the condenser consists of a hollow body, closed below and internally cooled, and preferably with a curved bottom, said body being disposed in a heated jacket in such a manner that the incoming vapors bathe the lowest portion of the cooling surface. This cooling tube is preferably provided with a device for maintaining a liquid or gaseous cooling medium in circulation therein, the arrangement being such that the heat is transmitted through the outer tube to the cooling medium principally by radiation. To enable the cooling action to be accurately regulated, it is advisable to arrange said circulating device so as to be vertically adjustable.

In order more clearly to understand the nature of the invention, reference is made to the accompanying drawings, which illustrate diagrammatically and by way of example, an embodiment of apparatus suitable for carrying out the process of the invention.

In said drawings Fig. 1 shows a front elevation in partial section; Fig. 2 a cross section; Fig. 3 a vertical section through a modified embodiment; and Fig. 4 a detail of a further modification.

Like reference characters denote like parts in the several figures of the drawings.

According to the embodiment shown in Figs. 1 and 2, the distillation chamber 1 is in the form of a tube which extends through a suitable heating apparatus, such as an electric radiation furnace 2. The material to be distilled is placed in a charging hopper 3 and passes through a lock chamber 4 having closure members 5 and 6 operable by levers, as shown, into a stock vessel 7, from which it is continuously fed, by means of a worm 8 or the like, into distillation chamber 1, through which the material is conveyed by means of a worm 9 or the like. The residue falls into a collector 10, from which it is discharged through a lock chamber 11 provided with closure members 5a and 6a. The collector 10 and chamber 11, as also the chamber 4 and stock vessel 7, are connected with a vacuum pump by means of pipes, as shown in Fig. 1, adapted to be closed independently.

Midway along its length the distillation tube 1 is connected by a conduit 12 with the outer shell 13 of a condenser, the discharge pipe 14 of which dips into a receiver 15. In the bottom of receiver 15 there is provided a valve 16. By arranging the condenser at a level more than 6 meters above the outlet level, a perfectly automatic barometric outlet device is obtained. This known arrangement can also be replaced by the 10 known double receiver for vacuum distillation, which enables work to be carried on without interruption by reversing devices.

In Fig. 4 there is illustrated such a double receiver which may be used in connection with the present process, and which is similar to that shown in Ullmann "Enzyklopaedie der Technischen Chemie" of 1929, second edition, third volume, at page 610. It comprises two receivers 45, 45a which may be connected alternatively by 20 means of the three-way valve 46 through pipe 14 to the condenser. Each of the receivers is adapted to be connected with the vacuum pump or the atmosphere by means of pipes controlled by valves 48, 48a, and 49, 49a, respectively. The 25 discharge pipes of the receivers 45 and 45a may be closed independently by valves 53 and 53a, respectively. Before the distillate is allowed to flow through the pipe 14 and the valve 46 to the receiver 45, the valve 48 will be opened to provide 30 a vacuum and the valves 49 and 53 will be closed. Simultaneously the distillate may be discharged from the receiver 45a; for this purpose, after closing the valve 48a and opening the valve 49a the valve 53a is opened. When the receiver 45a 35 is to receive the distillate and the receiver 45 is to be discharged the operation of the valves is reversed.

As shown in Fig. 2, the condenser consists of a cylindrical hollow vessel 17, closed below by a 40 curved bottom and disposed upright in a heated shell 13, in such a manner that the incoming vapors bathe the lowest portion of the cooling surface. A tube 18 is centered in the tube 17 so as to leave a small intermediate space all round 45 and allow the transmission of heat to take place principally by radiation, and tube 18 is cooled by means of a liquid or gaseous cooling medium, which is admitted through the tube 19a and passes away through the lateral branch 19b. The 50 whole of the circulation device is vertically adjustable in the tube 17, in order to enable the cooling action to be accurately regulated.

In order to remove accompanying dust, a filter is interposed in the pipe 12 connecting the chamber 1 with the condenser 13. The filtering medium consists preferably of loose, granular material, such as sintered magnesite or coal slack, disposed loosely in the connecting pipe. The arrangement shown in Fig. 2 has been adopted to 55 enable the filtering medium to be replenished without interrupting the work. The filtering medium 20 is disposed in a hopper 21, to the lower end of which is attached a tube 23, which can be closed by a valve 22 and dips into a collector 24, 60 whilst a pipe 25, leading from a stock vessel 26, rests on the heap. On the valve 22 being opened, the entire column of material is set in motion, the active portion becoming changed. If desired, the valve can be left slightly open all the time, so 65 that the changing is continuous. Since the filtering medium is more rapidly clogged up on the intake side than on the discharge side, it is advisable to arrange that the changing of the medium does not proceed with the same velocity on the 70 two sides. For this purpose a detroit member 75

is disposed, slightly eccentrically, in the hopper 21, so that the outlet passage on the intake side of the vapors is wider than the passage on the outlet side, and the medium accordingly moves more rapidly on the intake side than at the outlet side. 5

In order to direct the flow of the magnesium vapors, they are conducted to the condenser by means of a current of inert or reducing gas, such as hydrogen. For this purpose, supply pipes 28, 29, 30, 31 are employed, which, in the example 10 shown, are attached at both ends of the reaction chamber 1 (Fig. 1) and to the stock vessel 26 and outlet pipe 23 (Fig. 2), respectively.

The material to be distilled, such as magnesium dust furnished by the electrothermal reduction of 15 magnesium compounds, is heated in the heating zone to a temperature—according to the degree of vacuum—at which the magnesium already possesses a high vapor tension, preferably to a temperature near (slightly above) the boiling point. 20 The pipe 12 leading to the condenser (Fig. 1), the filter and the shell 13 of the condenser are heated to such an extent that the internal temperature can not fall below the solidification temperature of the magnesium. If the distillation be conducted within a pressure range of 50 to 200 mm. mercury gauge, the distillation tube and the other heated members of the device are maintained at a temperature between 850° and 1000° C. The actual cooling temperature of the condenser is 25 between 680° and 800° C.

According to the embodiment shown in Fig. 3, the horizontal reaction chamber is replaced by a vertical tube 32, forming the casing of one side of a bucket elevator 33. Before entering the heated 30 portion of the casing 32, the buckets 34 are filled with magnesium-containing material from a stock vessel 35 and this material is thereafter covered by filtering material discharged from a stock vessel 37. The outlets of each vessel are 40 adapted to be closed by slides 38, 39, respectively. The vapors generated in the heated section of the tube 32 pass through the filtering medium and are carried off to the condenser 13 by means of the 45 flushing gas admitted at 38 and 40. 45

Instead of conveying the material to be distilled through the distillation zone by means of a worm or bucket elevator, the process can also be carried out with the aid of other suitable known devices permitting the flow of the material under 50 the influence of gravity (such as for instance stationary furnaces comprising a series of hearths in step relation), or by rotation of a heated tube round its long axis (such as revolving furnaces), or by stationary furnaces provided with paddle-shaped conveying devices. It is only essential 55 that the magnesium-containing material pass through a heated zone so as to be brought to a temperature which causes transformation of the magnesium into the state of vapor, which temperature, of course, depends on the pressure conditions existing in the heated system, and that, after passing through a filter, the resulting magnesium vapor is subjected to such condensation 60 conditions that the metal will be converted to liquid form. 65

In all cases, heat-resisting special steels, free from nickel and copper, must be employed for constructing the apparatus of the present invention in order to prevent contamination of the resulting magnesium. 70

This application is a division of my copending application Serial No. 655,067, filed February 3, 75 1933.

According to the provisions of the patent statutes, I have explained the principle and mode of operating my invention, and have illustrated and described what I now consider to be its best embodiment. However, I desire to have it understood that, within the scope of the appended claim, the invention may be practiced otherwise than as specifically illustrated and described.

I claim:

A method of treating magnesium powder which comprises subjecting said powder to a temperature above the melting point, maintaining said powder in a continuous state of agitation to subject the same to a rubbing action, the temperature and pressure being such as to cause vaporization of magnesium, removing the vapors and condensing the same. 5

FRITZ HANSGIRG.